

## UNITED STATES PATENT OFFICE.

JOHN G. FUNCK, OF NEW ORLEANS, LOUISIANA.

## PLASTIC COMPOSITION.

1,268,000.

Specification of Letters Patent. Patented May 28, 1918.

No Drawing.

Application filed May 1, 1917. Serial No. 165,726.

*To all whom it may concern:*

Be it known that I, JOHN G. FUNCK, a citizen of the United States, residing at New Orleans, in the parish of Orleans and State of Louisiana, have invented certain useful Improvements in Plastic Compositions, of which the following is a specification, reference being had therein to the accompanying drawing.

- 10 The invention relates to a composition of matter for the manufacture of fence posts, telephone poles, uprights, window frames and similar materials as a substitute for wood.
- 15 The composition consists of the following ingredients combined in the proportions stated, viz:

|                  |                       |
|------------------|-----------------------|
| Lime             | 1/2 qt. or 2 parts    |
| Plaster of Paris | 1/2 qt. or 2 parts    |
| Cement           | 1 1/2 qt. or 5 parts  |
| Sand             | 3 1/2 qt. or 10 parts |

These ingredients are to be thoroughly

mingled by agitation or otherwise. The materials should be well sifted prior to the mixing thereof and the lime and plaster of Paris should be added dry when making the mixture, and in the mingling of the ingredients sufficient water should be added to render the mass soft.

After the mixing of the ingredients the mass should be poured into a mold or other former for the setting thereof and after the setting it is placed in the open for the thorough drying thereof.

Having thus described my invention, I claim:

A plastic composition for use as a substitute for wood consisting of about two parts by measure each of lime and plaster of Paris combined with approximately five parts of cement and ten parts of sand.

In testimony whereof I affix my signature.

JOHN G. FUNCK.

Copies of this patent may be obtained for five cents each, by addressing the "Commissioner of Patents, Washington, D. C."